

Sept. 7, 1937.

R. L. ADAMS

2,092,627

CARBON BRUSH

Filed April 27, 1935



Fig. 2.



Inventor:  
Roy L. Adams,  
by Harry E. Dunham  
His Attorney.

## UNITED STATES PATENT OFFICE

2,092,627

## CARBON BRUSH

Roy L. Adams, Schenectady, N. Y., assignor to  
 General Electric Company, a corporation of  
 New York

Application April 27, 1935, Serial No. 18,599

3 Claims. (Cl. 171—326)

The present invention relates to a method for joining copper to carbon and more particularly to carbon brushes for dynamo electric machines and a method for making the same.

5 One of the objects of the present invention is to provide a low resistance connection between a carbon brush and the flexible conductor usually employed to carry current to or from the brush.

The novel features which are characteristic of 10 my invention are set forth with particularity in the appended claims. The invention itself however will best be understood from reference to the following specification when considered in connection with the accompanying drawing in which 15 Fig. 1 is a view in elevation of a carbon brush embodying the features of my invention, while Fig. 2 is a cross sectional view of a modified form of my invention.

In carrying out my invention I apply a layer of 20 finely divided copper to a carbon block 1. The block and copper are then heated at an elevated temperature, for example about 600° C. to 800° C., but below the melting point of the copper, while pressure is simultaneously applied to the copper 25 to force it into the adjacent pores of the carbon and to weld the copper particles into a solid mass 2. During the heating process, any sulphur in the carbon block 1 rises to the upper surface thereof and forms a compound with a portion of 30 the copper providing thereby an intermediate layer 3 of copper sulphide. A flexible connector 4 may be secured to the welded copper mass 2 in a manner well known in the art.

Instead of applying pulverized copper to the 35 carbon block as hereinbefore indicated, it usually will be found preferable to apply a cupreous material such as pulverized copper sulphide directly to the carbon block and to heat the copper sulphide and carbon block to a 40 temperature of about 600° to 800° C. while pressure is simultaneously applied to the copper sulphide. An excess of copper sulphide is employed so that the adjacent pores of the carbon block will be 45 filled or impregnated and a layer of copper sulphide corresponding to layer 3 of Fig. 1 pro-

vided on top of the carbon. A copper plate corresponding to the welded copper mass 2 may then be secured to the layer of copper sulphide in any desired manner, for example by brazing, after which a flexible conductor 4 may be secured to 5 the copper plate. The intermediate layer of copper sulphide is secured to the carbon with such great tenacity that if an attempt is made to separate the copper sulphide from the carbon the break will occur in the carbon rather than at the 10 junction of the copper sulphide layer and the carbon.

Instead of applying finely divided copper or copper sulphide to the entire upper surface of the carbon block I may provide an opening in the upper surface of a carbon brush 5 and fill it with pulverized copper or copper sulphide 6 into which a flexible conductor 7 may be inserted after which pressure and heat may be applied to the pulverized material as hereinbefore set forth. 15

While my invention is particularly adapted for use in connection with commutator brushes it will be obvious that it is not limited to such use and that it may be employed in connection with carbon contacts and the like or in any device 20 where a particularly strong connection between copper and carbon is desired.

What I claim as new and desire to secure by Letters Patent of the United States, is:

1. A carbon block provided with a layer of copper sulphide thereon, the pores of said block adjacent said layer being impregnated with said sulphide. 30

2. A carbon brush provided with a layer of copper sulphide thereon, the pores of said brush adjacent said layer being impregnated with said sulphide, and a layer of copper on said layer of copper sulphide. 35

3. The method of forming a commutator brush which comprises applying pulverized copper sulphide to a carbon block, heating the block and copper sulphide at an elevated temperature, while pressure is simultaneously applied to the copper sulphide. 40

ROY L. ADAMS. 45